

# UNITED STATES PATENT OFFICE.

CLARENCE I. B. HENNING, OF WILMINGTON, DELAWARE, ASSIGNOR TO E. I. DU PONT DE NEMOURS & COMPANY, OF WILMINGTON, DELAWARE, A CORPORATION OF DELAWARE.

## PROPELLENT POWDER AND PROCESS OF MAKING SAME.

1,357,865.

Specification of Letters Patent.

Patented Nov. 2, 1920.

No Drawing.

Application filed March 3, 1920. Serial No. 363,105.

To all whom it may concern:

Be it known that I, CLARENCE I. B. HENNING, a citizen of the United States, and a resident of Wilmington, in the county of New Castle and State of Delaware, have invented a certain new and useful Propellant Powder and Process of Making Same, of which the following is a specification.

This invention relates to propellant powder compositions containing constituents capable of counteracting metallic fouling, and to a process of making such compositions.

The cause of metallic fouling, for which I have been successful in finding a remedy, may be briefly explained as follows: The introduction of breech loading in arms of all kinds led to giving rotation to the projectile by means of rifling with twists. As the chamber of the gun is larger than the bore, the projectile is provided with a soft metal band, usually of copper. When the combustion of the propellant powder causes the projectile to move forward, the bands of the projectile which conform in shape to the section of the rifling, assure the proper rotation to the projectile. As the band completely fills the cross section of the bore it also serves as a check to prevent the escape of gas past the projectile and in addition it serves to center the projectile in the bore and to determine a fixed position of the projectile when rammed in the gun. During the passage of the projectile through the bore of the gun the copper from the band fuses with the steel of the bore of the gun, due to the high temperature. This fouling of the bore of the gun is usually referred to as metallic fouling and the amount increases very rapidly as additional rounds are fired in the gun and soon reaches a point where the accumulated metallic fouling seriously affects the accuracy of the gun and also reduces the diameter of the bore of the gun to a point where the continued use of the gun is very dangerous because of developing too high pressure. It is, therefore, necessary after a relatively small number of rounds have been fired to either re bore or reline the gun.

I have previously explained in my application Serial No. 319,485, the serious effect of metallic fouling upon the accuracy and life of a gun or rifle, and have described and claimed therein the incorporation in the

nitrocellulose or nitrocellulose-nitroglycerin colloid of finely powdered metals, or a mixture of metals, or alloys, for reducing or removing the metallic fouling, thereby making possible a reduction in the amount of metallic fouling to one-third or one-fourth the usual amount occurring when using powder without the addition of a metal or alloy. Furthermore, the smaller amount of metallic fouling which is formed in the bore of the rifle or gun will be found to be more uniformly distributed in view of the fact that the metal or alloy is uniformly distributed throughout the propellant powder. This more uniform distribution of the metallic fouling in the bore of the gun taken with the smaller amount of metallic fouling formed decidedly improves the average accuracy of the gun or rifle and greatly prolongs its useful life. In addition to the material reduction in the amount of metallic fouling it has also been found that the muzzle flash is very much reduced, caused by the cooling effect of the metal or alloy on the gases, or for some other reason.

I have now made the additional discovery that instead of using the finely divided metals or mixtures of metals, or alloys, that I can substitute for these, in whole or in part, simple metalloid (i. e., nonmetal) derivatives, such as the oxids or salts, of metals capable of forming with the soft metal of the projectile an alloy which does not adhere as tenaciously to the bore of the gun at elevated temperatures as does the soft metal alone, this decreased powder of adhesion being characteristic usually of an alloy which is brittle at elevated temperatures.

My new propellant compositions and a process of making them may be illustrated by the following example:—

The improved propellant powder, containing, preferably in a finely powdered condition, oxids or salts of metals, according to my invention, can be made by a process similar to the usual process for making propellant powder for small arms and ordnance. For example, sufficient wet nitrocellulose to give 100 parts by weight of nitrocellulose, which may be a mixture of nitrocellulose soluble in ether-alcohol with nitrocellulose relatively insoluble in ether-alcohol, or may be a soluble nitrocellulose alone, is dehydrated with ethyl alcohol of approximately 110

2

95% by volume or 190 proof, by means of a dehydrating press, in order to displace the water. The excess alcohol is removed from the nitrocellulose, leaving about 33½ parts by weight of alcohol in the dehydrated nitrocellulose. To this is added approximately 60½ parts by weight of ethyl-ether in a suitable mixing machine, preferably provided with brine refrigeration. To the nitrocellulose and solvent in the mixer there may be added one-half or more parts diphenyl-amin or other stabilizer, with one to five or more parts of a metal oxid, such as finely powdered tin dioxid, together with other ingredients if desired, such as nitrocompounds, graphite, etc. The composition is thoroughly mixed and colloided, which operation in the mixer requires about ½ hour or more, depending on the efficiency of the mixer. After thorough mixing, the colloided composition is formed into preliminary blocks by means of a press. These blocks are then placed in a so-called finishing press, and the composition pressed 25 through dies into strings, which strings are granulated by means of a cutting machine. The granulated powder is then placed for one or more days in solvent recovery apparatus to recover alcohol and ether, and then 30 dried in water or air, to reduce the solvent remaining in the powder to a low amount. The powder is then air dried to remove excess surface moisture and may or may not be glazed.

35 Although the oxid of tin has been specifically mentioned above as a suitable compound for incorporation in the powder to counteract metallic fouling, there may also be used various other oxids, or salts, or 40 mixtures of oxids and salts, of those metals capable of forming with copper an alloy which is brittle at elevated temperatures. For example, there may be used, to advantage a mixture of approximately equal parts 45 by weight of tin dioxid with an oxygen derivative of lead, such as lead oxid or lead carbonate. Furthermore, the oxids or salts of the metals may be used in various combinations with each other or may be used in 50 combination with the finely powdered metals or mixtures of metals or alloys as set forth in my U. S. application Serial No. 319,485, above mentioned.

55 My invention is, furthermore, not limited to powder capable of overcoming the metallic fouling in connection with projectiles having a soft metal band composed of copper, but is also applicable to cases in which the soft metal band comprises a substance 60 other than copper either alone or in combination with copper. In any case whether the soft metal band consists entirely of copper or not, the finely divided oxids or salts of metals, or mixtures of oxids, and 65 salts with finely divided metal or metals, in-

corporated in the powder should be capable of forming with the soft metal of the band an alloy brittle at an elevated temperature and not adhering as strongly to the bore of the gun as does the soft metal alone. 70 For instance in small arms and munitions, the bullet is jacketed with an alloy of copper and nickel which according to usage in the United States is usually 85% copper and 15% nickel. My experiments indicate 75 that tin or tin oxid incorporated in the powder is efficient in removing the fouling from this cupro-nickel alloy, as well as metallic copper fouling. This is particularly important because the majority of military 80 small arms cartridges contain cupro-nickel jacket bullets.

I claim:—

1. The process of producing a propellant powder capable of counteracting the metallic fouling of the bore of a gun ordinarily caused by soft metal carried by the projectile to be shot from said gun, which comprises incorporating in a propellant powder composition a finely sub-divided metalloid derivative of a metal capable of forming with said soft metal an alloy which does not adhere as tenaciously to the bore of the gun at elevated temperatures as does the soft metal alone. 95
2. The process of producing a propellant powder capable of counteracting the metallic fouling of the bore of a gun ordinarily caused by soft metal carried by the projectile to be shot from said gun, which comprises incorporating in a propellant powder composition a metalloid derivative of a metal capable of forming with said soft metal an alloy which does not adhere as tenaciously to the bore of the gun at elevated 100 temperatures as does the metal alone. 105
3. The process of producing a propellant powder capable of counteracting the metallic fouling of the bore of a gun ordinarily caused by soft metal carried by the projectile to be shot from said gun, which comprises incorporating in a propellant powder composition a finely sub-divided oxid of a metal capable of forming with said soft metal an alloy which is brittle at elevated 110 temperatures. 115
4. The process of producing a propellant powder capable of counteracting the metallic fouling of the bore of a gun ordinarily caused by soft metal carried by the projectile 120 to be shot from said gun, which comprises incorporating in a propellant powder composition an oxygen derivative of a metal capable of forming with said soft metal an alloy which is brittle at elevated temperatures. 125
5. The process of producing a propellant powder capable of counteracting the metallic fouling of the bore of a gun ordinarily caused by soft metal carried by the projec- 130

- tile to be shot from said gun, which comprises incorporating in a propellant powder composition a finely divided metal oxid substance comprising tin dioxid.
6. A propellant powder containing a metalloid derivative of a metal capable of reducing metallic fouling.
7. A propellant powder containing in a finely divided condition a metalloid derivative of a metal capable of reducing metallic fouling.
8. A propellant powder containing in a finely divided condition an oxygen derivative of a metal capable of reducing metallic fouling.
9. A propellant powder containing in a finely divided condition an oxid of a metal capable of reducing metallic fouling.
10. A propellant powder containing uniformly distributed therethrough in a finely sub-divided condition a metalloid derivative of a metal capable of reducing metallic fouling.
11. A propellant powder containing uniformly distributed therethrough in a finely sub-divided condition an oxid of a metal capable of reducing metallic fouling.
12. A propellant powder containing uniformly distributed therethrough in a finely sub-divided condition an oxid of tin.
13. A propellant powder containing in a finely divided condition an oxid of tin.
14. A propellant powder containing in a finely divided condition an oxid of a metal capable of reducing metallic fouling and an oxygen derivative of lead.
15. A propellant powder containing uniformly distributed therethrough in a finely sub-divided condition tin dioxid and an oxygen derivative of lead.
16. A propellant powder containing from about 1 to 5% of a simple metalloid derivative of a metal capable of reducing metallic fouling.
- 48 17. A propellant powder containing from about 1 to 5% of a material comprising finely powdered tin dioxid.
18. A propellant powder containing from about 1 to 5% of a material comprising finely powdered tin dioxid and an oxygen derivative of lead.
19. A propellant powder containing, uniformly distributed therethrough in a finely divided condition, from about 1 to 5% of a material comprising an oxygen derivative of a metal capable of reducing metallic fouling.
20. A propellant powder containing, uniformly distributed therethrough in a finely divided condition, from about 1 to 5% of a material comprising lead carbonate and an oxygen derivative of another metal capable of reducing metallic fouling.
21. A nitrocellulose explosive grain containing in a finely divided condition a metalloid derivative of a metal capable of reducing metallic fouling.
22. A nitrocellulose explosive grain containing in a finely divided condition an oxid of a metal capable of reducing metallic fouling.
23. A nitrocellulose explosive grain containing in a finely divided condition an oxid of tin.
24. A nitrocellulose explosive grain containing uniformly distributed therethrough in a finely sub-divided condition tin dioxid and an oxygen derivative of lead.
25. A nitrocellulose explosive grain containing from about 1 to 5% of a material comprising finely powdered tin dioxid.
26. A nitrocellulose explosive grain containing, uniformly distributed therethrough in a finely divided condition, from about 1 to 5% of a material comprising lead carbonate and an oxygen derivative of another metal capable of reducing metallic fouling.

In testimony whereof I affix my signature.

CLARENCE I. B. HENNING.